

## 1

3,423,235

### ORGANOSILOXANE-CONTAINING FINISHES FOR ORGANIC FIBERS

James Kermit Campbell, Midland, Mich., assignor to Dow Corning Corporation, Midland, Mich., a corporation of Michigan  
No Drawing. Filed Nov. 23, 1964, Ser. No. 413,304  
U.S. Cl. 117—138.8 3 Claims  
Int. Cl. D06m 15/66



paraffin and hexane placed upon cotton and allowed to dry.

This application relates to organosiloxane-containing finishes for organic fibers.

Dimethylpolysiloxane is a known finish for organic fibers such as thread and yarn. It imparts superior and long lasting lubricity to the fibers, even when high temperatures and loads that would destroy organic finishes are generated on the fiber surface through friction.

For this reason dimethylpolysiloxane-finished threads and yarns are often used in high speed sewing and weaving machines where high friction can cause frequent fiber breakage is nonsilicone fiber finishes are used.

It would be desirable to dilute siloxane fiber finishes with organic oils and waxes to obtain improved lubricity over pure organic finishes at a reduced cost. Dimethylsiloxane, however, is incompatible with most organic oils and waxes, which makes it difficult to mix with organic materials.

It would further be desirable to develop waxy silicone fiber finishes, but in its usable forms dimethylpolysiloxane is a fluid. Waxy fiber finishes can be used to hold fibers together in a thread or yarn.

This application discloses new silicone compositions that possess the excellent fiber lubricating properties of dimethylpolysiloxane, yet which are compatible with almost all organic oils and waxes. When even minor quantities of the silicone of this application are added to organic oils and waxes, improved organic fiber finishes are obtained at low cost, showing superiority over nonsilicone fiber finishes.

The silicone compositions of this invention include waxy materials as well as fluids, and are superior to organic fiber finishes whether used alone or in combination with other materials.

This invention relates to the process of applying to an

## 2

organic fiber a composition comprising a polymeric siloxane consisting essentially of

(a)



10 units and

(b) at least one



unit per molecule, where R is an alkyl radical with an average of at least 14 carbon atoms and n has a value of 1 to 2, there being an average of from 1 to 12 (b) units for every 20 (a) units present, and there being an average of 4 to 100 (a) units per polymer molecule, whereby a lubricated fiber is formed.

25 R can be any alkyl radical of at least 14 carbon atoms such as the tetradecyl, octadecyl, eicosyl, and myricyl radicals. Compositions containing mixtures of R groups are acceptable for use in this invention.

If desired, the silicone of this invention can be diluted with an organic diluent in any proportion, though it is preferred to have at least one weight percent of the silicone of this invention present based on the weight of the diluted composition.

30 The organic diluent can be a material suitable for use as a fiber lubricant, e.g. any nondrying organic oil such as naphthenic base, paraffinic base, or mixed base petroleum lubricating oils, other hydrocarbon lubricants, such as lubricating oils derived from coal products and synthetic oils, e.g. alkylene polymers (such as polymers of propylene, butylene, etc., and mixtures thereof). Also,

35 alkylene oxide-type polymers, dicarboxylic acid esters, liquid esters of acids of phosphorus, alkyl aromatic hydrocarbons, and synthetic oils of the alkylene oxide-type polymers may be used, e.g. propylene oxide polymers produced by polymerizing propylene oxide in the presence of water or alcohols such as ethyl alcohol. Esters of

40 ethylene oxide-type polymers, such as acetylated propylene oxide polymers prepared by acetylating propylene oxide polymers containing hydroxyl groups, polyethers prepared from alkylene glycols such as ethylene glycol, fatty acid esters, and other organic oils are all suitable.

45 The polymeric products prepared from the various alkylene oxides and alkylene glycols may be polyoxyalkylene diols or polyalkylene glycol derivatives; that is, the terminal hydroxy group can remain as such, or one or

50 both of the terminal hydroxy groups can be removed during the polymerization reaction by esterification or etherification.

55 Synthetic oils of the dicarboxylic acid ester type include those which are prepared by esterification such dicarboxylic acids as adipic acid, azelaic acid, suberic acid, sebatic acid, alkenyl succinic acid, fumaric acid, maleic acid, etc., with alcohols such as butyl alcohol, hexyl alcohol, 2-ethylhexyl alcohol, dodecyl alcohol, etc. Examples

of dibasic (dicarboxylic) acid ester synthetic oils include dibutyl adipate, dihexyl adipate, di-2-ethylhexyl sebacate, di-n-hexylfumaric polymer.

Synthetic oils of the alkyl aromatic type include those which are prepared by alkylating benzene (e.g., dodecylbenzene, tetradecylbenzene, didodecylbenzene, etc.).

Polyhydric alcohol esters such as esters of trimethylol propane and pentaerythritol are also usable.

Organic waxes such as paraffin, beeswax, or carnauba wax can also be used as the diluent.

It may be desirable to use volatile solvents as part or all of the organic diluent to assist in the application of the composition to the fibers and to enhance the dispersability of the composition. Examples of suitable solvents are isopropanol, benzene, heptane, cyclohexane, acetone, diethylether, naphtha, trifluorotrichloroethane, dichlorobenzene and carbon tetrachloride.

Mixtures of organic diluents can be used. For example, to 5 weight percent of the silicone of this invention there can be added 45 weight percent of paraffin dissolved in 50 weight percent of heptane. A uniform, fluid dispersion will result that is easily applied to fibers, and which imparts superior lubricity.

It is preferred for the organic diluent, if present at all, to be present in the amount of 50 to 99 weight percent, based on the total weight of the composition, and for essentially all of the rest of the composition to be the silicone of this invention.

If R has an average of at least 20 carbon atoms, the silicones of this invention will tend to be waxy, which is preferred. If R has an average of less than 20 carbon atoms, the silicones of this invention will tend to be fluids, which may be desirable in many circumstances.

The silicones of this invention can be made by equilibrating octamethylcyclotetrasiloxane and



in the known manner by means of an acid catalyst such as sulfuric acid, wherein n has a value of approximately 5-40. Both of these silicone materials are commercially available from the Dow Corning Corporation of Midland, Mich.

The product will be a copper of dimethylsiloxane and methylhydrogensiloxane. The ratio of the two units to each other is controlled by the ratio of the initial ingredients; the product should have from 1 to 12



units for every 20



units present, and the degree of polymerization should not exceed 100



units per molecule, preferably there being no more than 40 of such units per molecule. The degree of polymerization can be controlled by the amount of endblocking units that are present, e.g.  $[(CH_3)_3SiO -]$ .

The above copolymeric product is then reacted with 5 one or more types of alpha olefin having an average of at least 14 carbon atoms per molecule, the reaction being in the presence of a platinum catalyst with heating to about 100 to 150° C.

The product will be a copolymer of



where R is defined above. This is the silicone of this invention.

Another method of making the silicones of this invention is to equilibrate octamethylcyclotetrasiloxane with



in the presence of a catalyst such as NaOH. The above disiloxane can be made by reacting tetramethyldisiloxane with the appropriate alpha olefine in the presence of platinum.

The products made by this particular process possess higher alkyl groups only on the terminal silicon atoms of each molecule.

The fluid compositions of this invention can be applied 40 to fibers by means of spraying, running the fibers over a pad soaked with the composition, or any other known way of applying fluids to fibers. The waxy compositions of this invention can be applied by melting the composition to the fluid form and then applying it, or by running the fibers across the waxy substance, etc.

Any organic fiber can be used in this invention. For example, any yarn or thread made of wool, cotton, rayon, hemp, silk, polypropylene, polyesters such as Dacron®, polyamides such as nylon, polyethylene, or cellulose acetate is operative.

The greatest improvements in lubricity tend to occur when cellulosic fibers such as cotton, or acrylic (polyacrylonitrile) fibers are used.

The following examples are illustrative only and should 55 not be construed as limiting the invention, which is properly delineated in the appended claims.

#### EXAMPLE 1

Various yarns were treated with 10% toluene solutions of various silicone finishing agents to achieve 1.0% solids on the yarn, based on the weight of the yarn, and allowed 60 to dry.

These yarns were then tested for frictional characteristics against either a ceramic or steel spindle. The yarn was looped over the spindle with a tension at rest of about 80 grams. During the test the yarn traveled over 70 the spindle at 100 yards per minute. Two strain gauges recorded the difference in tension on the yarn before and after passing the spindle to yield a relative measure of the frictional force between the yarn and the spindle. This relative friction was expressed as a number, the 75 lower frictions being expressed by lower numbers.

The results are shown below:

| Finishing agent for yarn                                                                                                                                                                                                                                                             | Relative friction |                 |               |                 |
|--------------------------------------------------------------------------------------------------------------------------------------------------------------------------------------------------------------------------------------------------------------------------------------|-------------------|-----------------|---------------|-----------------|
|                                                                                                                                                                                                                                                                                      | Cotton yarn       |                 | Acrylic yarn  |                 |
|                                                                                                                                                                                                                                                                                      | Steel spindle     | Ceramic spindle | Steel spindle | Ceramic spindle |
| None                                                                                                                                                                                                                                                                                 | 12                | 12              | 20            | 4               |
| $\begin{array}{c} \text{CH}_3 \quad \text{CH}_3 \quad \text{CH}_3 \\   \quad   \quad   \\ \text{R} \text{SiO}(\text{SiO})_{4-n} \text{SiR} \quad \text{R} = \text{C}_{22} \text{ and above} \\   \quad   \quad   \\ \text{CH}_3 \quad \text{CH}_3 \quad \text{CH}_3 \end{array}$     | 7                 | 7               | 4.5           | 5               |
| $\begin{array}{c} \text{R} \quad \text{CH}_3 \\   \quad   \\ (\text{CH}_3)_3\text{SiO}(\text{SiO})_3(\text{SiO})_{24}\text{Si}(\text{CH}_3)_3 \quad \text{R} = \text{C}_{22} \text{ and above} \\   \quad   \\ \text{CH}_3 \quad \text{CH}_3 \end{array}$                            | 7                 | 7               | 4.5           | 5               |
| $\begin{array}{c} \text{CH}_3 \\   \\ (\text{CH}_3)_3\text{SiO}(\text{R SiO})_3(\text{SiO})_{24}\text{Si}(\text{CH}_3)_3 \quad \text{R} = \text{C}_{18} \\   \quad   \\ \text{CH}_3 \quad \text{CH}_3 \end{array}$                                                                   | 8                 | 8               | 5.5           | 8               |
| $\begin{array}{c} \text{CH}_3 \quad \text{CH}_3 \\   \quad   \\ (\text{CH}_3)_3\text{SiO}(\text{R SiO})_3(\text{SiO})_3(\text{SiO})_{24}\text{Si}(\text{CH}_3)_3 \quad \text{R} = \text{C}_{14} \\   \quad   \quad   \\ \text{CH}_3 \quad \text{CH}_3 \quad \text{CH}_3 \end{array}$ | 10                | 12              | 6             | 8.5             |
| $\begin{array}{c} \text{CH}_3 \\   \\ (\text{CH}_3)_3\text{SiO}(\text{R SiO})_{35}\text{Si}(\text{CH}_3)_3 \quad \text{R} = \text{C}_{18} \\   \\ \text{CH}_3 \end{array}$                                                                                                           | 1                 | 11              | 8             | 8               |
| Dimethylpolysiloxane*, 350 cs                                                                                                                                                                                                                                                        | 9                 | 8               | 5.5           | 8               |

\*This composition is outside of the claims of this invention, and is shown for comparison.

### Example 2

When a dispersion of 10 grams of



35

20 grams of paraffin, and 40 grams of hexane is placed on a cotton thread and allowed to dry, the lubricity of the thread is greatly enhanced, and the heat stability of the lubricating coat is greater than that of a cotton fiber coated with paraffin alone.

### Example 3

When a dispersion of 10 g. of



45

40 grams of paraffin, and 40 grams of dibutylether is placed on a nylon yarn, the strands of the yarn adhere together after drying, while the nylon to nylon friction between various pieces of the yarn is considerably reduced.

That which is claimed is:

1. An organic fiber having coated thereon a lubricating composition consisting essentially of  
(1) from 1 to 50 weight percent of a polymeric siloxane consisting essentially of

(a)



units, and

(b) at least one



unit per molecule, where R is an alkyl radical with an average of at least 14 carbon atoms, and

n has a value of 1 to 2,

there being an average of 1 to 12 (b) units for every 20 (a) units present, and there being an average of 4 to 100 (a) units present per polymer molecule, and

(2) from 99 to 50 weight percent of a compatible diluent selected from the group consisting of non-drying organic oil and wax.

2. The article of claim 1 wherein the fiber is cotton.

3. The article of claim 1 where the fiber is acrylic.

### References Cited

#### UNITED STATES PATENTS

- |           |         |               |             |
|-----------|---------|---------------|-------------|
| 2,486,162 | 10/1949 | Hyde          | 260—448.2 X |
| 2,698,817 | 1/1955  | Guenther      | 117—138.8   |
| 2,735,791 | 2/1956  | Peyrot et al. | 117—138.8 X |
| 2,872,356 | 2/1959  | Bull et al.   | 117—139.5   |
| 3,187,752 | 6/1965  | Glick         | 117—138.8 X |

60 WILLIAM D. MARTIN, Primary Examiner.

J. E. MILLER, JR., Assistant Examiner.

U.S. Cl. X.R.

117—143, 139.5, 167, 168